

Nov. 20, 1923.

1,474,953

R. E. BRADLEY ET AL

## METHOD FOR TREATING METAL

Filed June 17, 1922



*Inventors:*  
*Ross Edward Bradley*  
*and Charles Raymond Webber;*  
*By* *Notoroadele*  
*Attorney.*

## UNITED STATES PATENT OFFICE.

ROSS EDWARD BRADLEY AND CHARLES RAYMOND WEBBER, OF BALTIMORE, MARYLAND, ASSIGNORS TO BALTIMORE TUBE COMPANY, INC., OF BALTIMORE, MARYLAND, A CORPORATION OF VIRGINIA.

## METHOD FOR TREATING METAL.

Application filed June 17, 1922. Serial No. 568,924.

*To all whom it may concern:*

Be it known that we, ROSS EDWARD BRADLEY and CHARLES RAYMOND WEBBER, residents of Baltimore, county of Baltimore, 5 State of Maryland, have invented a new and useful Method for Treating Metal, of which the following is a specification.

Our invention relates to improvements in method and means for the treatment of 10 metal bodies composed of copper or brass, or other alloys, and is especially adapted for the treatment of tubes.

The object is to cause such readjustment 15 of the metal particles or grains as to fit the metal body for the service for which it is intended. The invention also comprises method and means for confining the treatment of the metal body to a specific part of the said body, leaving the other parts thereof 20 unaffected by such treatment, thereby preserving to each part the characteristics which especially qualifies it for the service required of such part.

It is well known that brass and copper 25 tubes of certain uniform grain structure give longer life in service than other tubes. This grain structure is obtained ordinarily by annealing in an annealing furnace the tube, which has been previously hard drawn. 30 The annealing furnace, which is usually oil fired, but in some cases heated by other heating mediums, gives very erratic results so far as uniform grain structure is concerned.

By the method comprised in the present 35 invention, an electric current is passed through that portion of the metal body only, the structure of which it is desired to change or modify. This is accomplished by attaching the terminals to certain points on 40 the body, so that only the intervening space between said points shall be affected by passing the current therethrough. The time, amperage, voltage and cycle of alternation, where alternating current is used, are accurately regulated with respect to the cross- 45 section and composition of the portion of metal body treated, and recrystallization desired. The passage of the electric current through the metal body treated, causes a thermal expansion of the metal. This thermal expansion of the metal body is preferably utilized for automatically determining the time of current flow. This automatic expansion control may therefore be utilized,

in combination with the proper regulation 55 of amperage, voltage, etc. so that a complete recrystallization, to the predetermined grain size between the points of connection, can be effected.

In other words, by a proper correlation 60 of the coefficient of expansion of the metal body, under given conditions of voltage, amperage, cycle, etc. it is possible to utilize the said expansion after a predetermined period of said current flow, automatically 65 to break the current, and the predetermined period may be adjusted to secure the grain structure desired.

It will thus be seen that upon the predetermined expansion may be accurately correlated 70 these factors; amperage, voltage, cycle of alternation, cross-section of metal body, and time of current flow.

The invention is peculiarly applicable to 75 the treatment of brass or admiralty tubes for condensers. By locating the terminals at specific points on the tube extension, it is possible to eliminate what is known as "necking" or "crushing" of the tube, when 80 packing in the crown sheet of the condenser. It is possible by this method to leave the ends, where the packing is applied of sufficient hardness, or entirely hard, to resist 85 this crushing action, and at the same time to effect a complete reformation, as to size and arrangement of the grain of the metal between said points.

Referring to the drawing, which represents, merely by way of example, suitable 90 means for effecting our invention;

Fig. 1 is a view in elevation;

Fig. 2 is a cross-section on line 2, 2 of Fig. 1, on an enlarged scale;

Fig. 3 is a view made from a micro-photograph of a section of the metal before treatment;

Fig. 4 is a similar view showing the granular formation, after treatment in accordance with our invention.

Similar numerals refer to similar parts 100 throughout the several views.

The following is a specific example of the treatment of a brass tube in accordance with our invention.

The tube 5, which is 17.0 feet long, and  $\frac{1}{2}$  105 inches in diameter, with a .050 inch thick wall, is secured in the clamp brackets 6 and 7. The brackets 6 and 7 are connected to the

bus bars 8 and 9 which are connected through the switch board 10 with the transformer 11. The clamping bracket 6 has a fixed relationship with bus bar 8, while 5 clamping bracket 7 has a movable relationship with bus bar 9. The tube 5 which is to be treated is clamped in brackets 6 and 7 with its ends projecting beyond said brackets. The switch board 10, is provided with 10 a number of switches or controllers 13, for controlling, and the several meters 14, for indicating the character of current flow. The current is also controlled by an automatic circuit breaker, as at 15. This circuit breaker is provided with coils 16 connected to contacts 17 adapted to be bridged by the bridge 18 on frame 19 connected to the movable clamp bracket 7.

In operation: The tube is clamped in position, as above indicated, with the movable clamp bracket so positioned with respect to the contacts 17, as to require an exact predetermined movement of the bracket, due to the thermal expansion of the tube, to cause 25 the bridging of the contacts 17.

The circuit is then closed, with the section or extension of tube 5, between points or brackets 6 and 7, acting as a resister in said circuit. The current is so controlled by the 30 usual controlling devices, as to maintain it at approximately 3250 amperes, 32 volts, 25 cycles; the time of treatment required is from five to six seconds and the temperature of the tube approximately 800° F.

As a result of these factors the tube of 35 form and character above specified will have an expansion of approximately 1½ inches between the initial positions of brackets 6 and 7. This will cause at the moment of required expansion, the movement of bracket 40 7, sufficient to bridge the contacts 17, whereupon the circuit is interrupted and the process of treatment is completed.

As the result of such treatment, the part 45 of the tube, extending between points 6 and 7, will become perfectly uniform and homogeneous in grain structure, as indicated in Fig. 4, and of maximum cohesion, resulting in a tough and malleable body adapted to 50 give the greatest possible service as a condenser tube, while the end extensions of tube 5 beyond, or outside of the points 6 and 7, will remain hard, that is, unaffected by the current, so as to resist the necking or crushing 55 stresses when packing in the crown sheet.

What we claim is:—

1. The method of treating tubes composed of copper or the alloys of copper, which consists in subjecting the same to 60 an electric current, under relative conditions of voltage and amperage substantially as specified, and co-relating the expansion of the metal treated, and the period of current flow, substantially as described.

2. The method of treating tubes composed of copper or the alloys of copper, which consists in subjecting the same between points removed from its two ends to an electric current, under relative conditions of voltage and amperage substantially as 70 specified, and co-relating the expansion of the metal treated, and the period of current flow, substantially as described.

3. The method of treating tubes composed of copper or the alloys of copper, which 75 consists in subjecting the same to an electric current, under relative conditions of voltage, amperage and cycle, substantially as specified, and co-relating the expansion of the metal treated, and the period of current flow, substantially as described. 80

4. The method of treating tubes composed of copper or the alloys of copper, which consists in subjecting the same to an electric current, under relative conditions of voltage and amperage, substantially as specified, and co-relating the expansion of the metal treated, and the period of current flow, substantially as specified, to secure the 85 desired reformation of grain structure, substantially as shown. 90

5. The method of treating tubes of copper or the alloys of copper, which consists in subjecting the same to an electric current, and co-relating the expansion of the metal 95 body, under relative conditions of voltage and amperage substantially as specified, and utilizing the direct action of said expansion, after a predetermined period of said current flow, to interrupt said current 100 flow. 100

6. The method of treating tubes of copper or the alloys of copper, which consists in subjecting the same to an electric current, and co-relating the expansion of the metal body, under conditions of voltage and amperage substantially as specified, and utilizing the direct action of said expansion, after a predetermined period of said current flow, to interrupt said current flow, and adjusting said predetermined period of flow in order to secure the grain structure 105 desired. 110

7. The method of treating tubes of copper or the alloys of copper, which consists in subjecting the same to an electric current of approximately 3250 amperes, 32 volts and 25 cycles, and co-relating the content and expansion of the metal body, and utilizing the direct action of said expansion, after a predetermined period of said current flow to interrupt said current flow, and adjusting said predetermined period of flow in order to secure the grain structure 115 desired. 120

ROSS EDWARD BRADLEY.  
CHARLES RAYMOND WEBBER.